

J. IRVING.

PROCESS FOR TREATING ORES.  
APPLICATION FILED JAN. 27, 1917.

1,296,523.

Patented Mar. 4, 1919.



Inventor

Joseph Irving  
John and Augustus  
his Attorneys

# UNITED STATES PATENT OFFICE.

JOSEPH IRVING, OF BISBEE, ARIZONA.

## PROCESS FOR TREATING ORES.

1,296,523.

Specification of Letters Patent.

Patented Mar. 4, 1919.

Application filed January 27, 1917. Serial No. 144,890.

To all whom it may concern:

Be it known that I, JOSEPH IRVING, of Bisbee, in the county of Cochise and State of Arizona, have invented certain new and useful Improvements in Processes for Treating Ores; and I do hereby declare the following to be a full, clear, and exact description of the invention, such as will enable others skilled in the art to which it appertains to make and use the same.

My invention relates to a process for the treatment of cupriferous ores, compounds or products for the extraction of the metal values therefrom in soluble form and for the recovery of these metal values. Its objects are to effect in such a process a continuous regeneration of the reagents, the presence of which is desired, and simultaneously to eliminate undesirable reagents to avoid waste, and to reduce the amount of added chemicals required to a minimum, and to render the process cyclic in all its parts in so far as is possible. Further objects of my invention will more fully herein-after appear.

In carrying out my invention I have applied it to the treatment of copper ores, compounds or products, by wet extraction of the metal values therefrom by means of a solvent or electrolyte, subsequently subjecting this electrolyte containing the dissolved metal values to a treatment including an electrolytic precipitation for the separation of the metal values therefrom and for the simultaneous regeneration within the electrolyte of those compounds which make it effective as a solvent. I then repeat the cycle of operation upon fresh ore, using the regenerated electrolyte or solvent for this purpose. I have also provided therein for the formation within the solution of depolarizing agents prior to and during the electrolytic precipitation as well as for the regeneration of solvent chemicals therein. Furthermore I have provided in my process for the continuous production and regeneration of solvent washing solutions and have thus reduced to a minimum the addition of useless liquid during the cycle of operation.

In treating a cupriferous ore, for example, a low grade carbonate ore, I first grind the ore to a suitable degree of fineness and subject it to the action of the solvent or electrolyte. I may grind the ore

dry in a crushing plant and send it to the mixer, where it is mixed with the required amount of solvent or electrolyte, or I may grind it wet with a small amount of the solvent or electrolyte and send it to the mixer, where sufficient electrolyte is added to bring the total quantity of electrolyte solvent to the required amount.

The electrolyte, when used at this point as a solvent, is derived from the electrolytic copper precipitation tanks at a subsequent step in the process, and is a dilute solution containing as its principle actively solvent ingredients sulfuric acid and ferric sulfate. It is apparent, of course, that in initially installing my process it may be necessary to use a dilute solution containing sulfuric acid as the primary solvent, but once the process is set in operation, the electrolyte from the copper precipitation tanks becomes available, and the active components are substantially as above set forth. The proportions of the ingredients of the electrolyte are variable to a considerable extent, being dependent upon the conduct of the steps of the process subsequent to the extraction of the ore, the requirements of the precipitation bath, etc. I have found, however, that a suitable working strength is an acid concentration of about 1%  $H_2SO_4$  by weight and that a suitable proportion of electrolyte to ore in the case of the copper carbonate ore mentioned is about 300 gal. of solvent per ton of ore.

After the electrolyte or solvent and the ore have been in contact in the mixers while subjected to mechanical agitation for a sufficient length of time, the pulp and sand are run into suitable classifying and separating devices, preferably continuous flow devices in which separation may be effected simultaneously with a washing of the solid present by a counter current of solvent. I may use, for example, a series of displacement tanks, or counter current overflow thickeners of the Dorr type, or other like devices. Thus, for example, I may pass the pulp from the mixers first to a suitable settling tank or classifying machine, where the sands are separated from the pulp. The pulp is then passed to a series of thickening devices, in which a further washing or leaching is effected. The separated sands are further leached and washed with a suitable quantity of fresh electrolyte or solvent,

which, after being separated from the sands, is added to pulp first separated therefrom while flowing from the settling tanks or classifying machines, and passes with it 5 through the subsequent thickening and washing steps.

Further washing of the sands is effected by means of the solution obtained from iron precipitation tanks on passing portions of 10 electrolyte containing copper over metallic iron. The solution is brought into intimate contact with the sands, the ferric sulfate therein acting to leach out all undis- solved copper possible. The solution is 15 then returned to the iron precipitation tanks after being passed through a copper pyritic filter in which any ferric sulfate remaining in the solution is reduced to ferrous sulfate, copper being at the same time dissolved. In 20 this way a closed circuit of the washing solution is maintained, the continual addition of water is avoided, and the amount of liquid necessary for the operation of the process is reduced to a minimum. The 25 sands, after this washing, are discharged as tailings.

I may next subject the pulp from the settling tanks, to which the solution derived from the first washing of the sands by elec- 30 trolyte solvent has been added, to a treatment adapted to effect a separation of the liquid therein from the solids and to wash the separated solids. This I may effect, for example, by a series of gravity, counter 35 current thickeners, displacement tanks or other suitable devices, preferably arranged in two groups of one or more each. In the first group I effect substantially completely the separation of the slimes or solid ma- 40 terials in concentrated form from the solution, now carrying the metal value of the ore in solution, and I then pass the concentrated slimes into the second group for washing, while the solution is passed to the 45 electrolytic precipitation system.

In passing the concentrated slimes into the second group of thickeners or other selected devices I add thereto a sufficient quantity of the solution obtained from iron 50 precipitating tanks to cause a continuous flow through this group. Water may also be added at this point to reduce the concentration of the liquid when necessary. I thereby effect a further concentration of the 55 slimes and at the same time wash or leach them, further depriving them of any copper contained therein by virtue of the solvent action of the ferric sulfate in the solution added. The washed and concen- 60 trated slimes are now discharged as tailings and the washing solution is passed through the copper pyrites filter bed, thereby ex- hausting the solvent power of any ferric sulfate remaining therein and is returned 65 to the iron precipitation tanks.

In this way, as in the case of the wash- 70 ing solution for the sands described above, there is a closed circuit of the washing solution with all the advantages derived therefrom. Both washing solutions are thus taken from the iron precipitation tanks and after use returned thereto.

The electrolyte or solution obtained from the first group of thickeners is next passed through a filter of finely ground copper 75 pyrites. By this means any ferric sulfate remaining in the electrolyte is reduced to ferrous sulfate, copper and iron being dissolved therein. From the copper pyrites filter the solution passes to a sump tank, 80 where any slimes present are allowed to settle out. From here the electrolyte is sent to a series of alternately arranged reducing cells and electrolytic cells to effect the deposition of the copper and other metal 85 values.

In the reducing cells the electrolyte is brought in contact with the copper precipitate obtained from the iron precipitation system or from an outside source for the 90 purpose of reducing any ferric sulfate present to ferrous sulfate. The ferrous sulfate serves in the electrolytic cells as a depolarizing agent, and is therein oxidized to ferric sulfate. By the use of a series of alternat- 95 ing reducing and electrolytic cells and caus- 100 ing a continuous flow of the copper bearing electrolyte therethrough, the ferric sulfate formed by anodic oxidation in each electrolytic cell is reduced by the copper precipitate in the succeeding reducing cell, copper being dissolved, and the electrolyte passes into the next electrolytic cells with its depolarizer regenerated and a somewhat in- creased copper content. The copper dis- 105 solved is then deposited. The sulfuric acid formed in the electrolytic cells also dissolves additional copper in the reducing tanks, and thus is prevented from becoming too concentrated. The number of reducing and 110 electrolytic cells may vary as found desirable. I have found a series of two or three of each to effect a satisfactory deposition of the copper. By arranging the cells in successive order I provide for a continuous 115 flow of the electrolyte through the entire system.

The final electrolytic cell of the series I 120 purposely construct of extra large size in order to increase to some extent the anodic oxidation and the formation of ferric sulfate in the electrolyte, although cathodic efficiency is thereby slightly diminished. In the series of electrolytic cells the copper con- 125 tent of the electrolyte is reduced to about two per cent., this being the minimum quantity necessary for successful operation. From the last cell of the series of reducing and electrolytic cells the depleted electrolyte flows into a sump or settling tank, from 130

which it is returned to the starting point of the process to be mixed with ore and to leach the same.

- 5 While in the sump tank the sulfuric acid concentration of the electrolyte is, if necessary, brought to the point most suitable for leaching the ore by the addition of sulfuric acid. If the electrolyte is found to be deficient in sulfate of iron, a part of it, in 10 passing from the tank to the ore leaching apparatus, is diverted through a bed of finely ground pyrites, whereby its content of iron sulfate is increased to the desired point.
- 15 In case the electrolyte becomes foul, that is, accumulates so large an amount of foreign salt or of salts necessary for the operation of the process as to interfere with the operation thereof, I cause a part of the 20 electrolyte to pass into the iron precipitating system, where it is passed over metallic iron.

The copper in the electrolyte is thereby precipitated and the solution containing foreign salts may be discharged as waste, or caused to pass into the secondary washing solution used in the final washing of the sands or pulp, as hereinbefore described. The electrolyte may then be replenished, if 25 necessary, with dilute acid of a suitable concentration. The copper here obtained is used in the reducing cells arranged in series with the electrolytic cells, where it is redissolved in reducing the ferric sulfate, to 30 be subsequently redeposited. If it is desired to increase the amount of copper precipitate resulting after precipitation in the iron precipitating system I may divert thereto a part of the solution obtained by 35 the primary leaching of the ore with electrolyte.

It is apparent from the above description of my process that in it I have provided for a continuous flow of the working solution 40 in such a manner as to extract the metal values from the ore, remove them and return the solution to the work of extraction on the ore, and have also provided that at each step in the process the solution be 45 brought to a state whereby its efficiency in carrying out the next step is a maximum. Furthermore I have provided not only that the working solution be maintained in a closed circuit, but also that the various washing solutions used are maintained in closed 50 circuits. I have thereby reduced the necessity of cumulative additions of water and other inert materials to a minimum and have brought the amount of waste to the lowest 55 possible degree.

My process readily adapts itself for the treatment of copper ores containing gold or silver. In such case I effect the primary leaching of the ore with the electrolyte as 60 obtained from the copper depositing tanks

and the separation thereof from the sands and slime in the same manner as above described. The sands and slimes in this case also I wash with the solution yielded by the iron precipitation tanks, but add thereto a 70 quantity of salt. The resulting solution of chlorides and sulfates acts to dissolve the gold and silver values in the sands and slimes, as well as to wash out the undissolved copper. This washing solution is returned in the cycle as previously described to the iron precipitation tank, when the gold and silver value are precipitated together with the copper to form the copper precipitation which is used in the reducing 75 cells which alternate with the electrolyte cells. The copper is here dissolved, but the gold and silver are left undissolved in the sludge and are thus recovered.

My process as above described is illustrated by the flow sheet shown in the accompanying drawing. In this drawing the steps in my process wherein only a portion of a material is treated are indicated by dotted flow lines and the reagents added in 80 recovering precious metals are indicated by surrounding the same with circles.

I claim as my invention:

1. In the treatment of cupriferous ores, compounds or products, subjecting the ore 95 to the action of iron-containing electrolyte from the copper depositing tanks, removing the electrolyte and removing the copper therefrom, washing the treated ore with an iron-containing solution, passing the said 100 solution over iron, thereby reducing the iron salts contained therein and precipitating copper therefrom, and again washing treated ores with the said solution.

2. In the treatment of cupriferous ores, 105 compounds or products, subjecting the ore to the action of iron-containing electrolyte from the copper depositing tanks, removing the electrolyte, washing the thus treated ore with an iron containing solution, then 110 passing said solution over iron, thereby reducing the iron salts contained therein and precipitating copper therefrom, removing said copper and treating the electrolyte from the treatment of the ore therewith, thereby 115 reducing the iron content of said electrolyte and dissolving the copper, and depositing the copper in said electrolyte electrolytically.

3. In the treatment of cupriferous ores, 120 compounds or products subjecting the ore to the action of iron-containing electrolyte from the copper depositing tanks, removing the electrolyte, washing the thus treated ore with an iron containing solution, then 125 passing said solution over iron, thereby reducing the iron salts contained therein and precipitating copper therefrom, removing said copper and treating the electrolyte from the treatment of the ore therewith, thereby 130

- reducing the iron content of said electrolyte and dissolving the copper, depositing the copper in said electrolyte electrolytically and again treating ore with the electrolyte 5 thus obtained.
4. In the treatment of cupriferous ores, compounds or products, subjecting the ore to the action of the iron-containing electrolyte from the copper depositing tanks, reducing 10 the iron salts contained therein, depositing the copper therefrom electrolytically and thereby re-oxidizing the iron contained therein, increasing the iron content of the electrolyte and then again treating ore with 15 the resulting liquid.
5. In the treatment of cupriferous ores, compounds or products, subjecting the ore to the action of the iron-containing electrolyte from the copper depositing tanks, 20 passing said electrolyte through a pyritic filter, depositing the copper therefrom electrolytically, and thereby reoxidizing the iron contained there, passing a portion of said electrolyte through pyrites, thereby in- 25 creasing the content of iron salts therein and causing it to rejoin the remainder of the electrolyte, and again treating ore with the resulting liquid.
6. In the treatment of cupriferous ores, 30 compounds or products, subjecting the ore to the action of iron-containing electrolyte from the copper depositing tanks, reducing the iron salts contained therein, depositing the copper therefrom electrolytically and thereby re-oxidizing the iron contained 35 therein, passing a part thereof over metallic iron and replenishing the volume of the electrolyte, thereby diminishing its content of foreign salts, again treating the ore with 40 the resulting liquid, and utilizing the liquid resulting from the precipitation with iron to wash ore previously treated with electrolyte.
7. In the treatment of cupriferous ores, 45 compounds or products, subjecting the ore to treatment with an iron-containing solvent, separating the solvent therefrom, subjecting the separated solvent to a reducing reagent, subsequently precipitating the copper elec- 50 trolytically therefrom under conditions adapted to cause oxidization of the iron content thereof, and subsequently treating ore with the solvent thus obtained.
8. In the treatment of cupriferous ores, 55 compounds or products, subjecting the ore to treatment with an iron-containing solvent, separating the solvent therefrom, repeatedly subjecting the separated solvent alternately to a reducing reagent, and to the action of
- an electric current to effect deposition of the 60 copper, the final electrolytic treatment being under conditions adapted to effect a relatively extensive oxidation of the iron content thereof, and subsequently treating ore with the solvent thus obtained. 65
9. In the treatment of cupriferous ores, compounds or products, subjecting the ore to treatment with an iron-containing solvent, separating the solvent therefrom, washing the treated ore with an iron-containing solution, 70 passing said washing solution over iron, thereby precipitating copper therefrom and regenerating the washing solution for further use in washing and leaching ore, subjecting the first solvent alternately to the 75 action of an electric current and to the copper-iron deposit from the washing solution, and finally to an electrolytic treatment adapted to effect a relatively extensive oxidation of the iron content, thereby regenerating the solvent for reuse in treating 80 fresh ore.
10. In the treatment of cupriferous ores, compounds or products, containing precious metals, subjecting the ore to the action of 85 iron-containing electrolyte from the copper depositing tanks, removing the electrolyte, washing the thus treated ores with a solution containing iron and chlorides, then passing said solution over iron, thereby reducing the 90 iron contained therein and precipitating copper and the precious metals, and again washing treated ores with the said solution.
11. In the treatment of cupriferous ores, compounds or products, containing precious 95 metals, subjecting the ore to the action of iron-containing electrolyte from the copper depositing tanks, removing the electrolyte, washing the thus treated ore with a solution containing iron and chlorides, then passing 100 said solution over iron, thereby reducing the iron contained therein and precipitating copper and the precious metals, removing the precipitate and treating the electrolyte from the treatment of the ore therewith, thereby 105 reducing the iron contained in said electrolyte and dissolving the copper, recovering the precious metals from the residual sludge and depositing the copper in said electrolyte electrolytically. 110
- In testimony whereof, I have signed this specification in the presence of two subscribing witnesses.
- JOSEPH IRVING.
- Witnesses:
- CLIFTON MATHEWS,  
JEAN BOYD.